

## UNITED STATES PATENT OFFICE

2,608,482

FERROCHROME-SILICON-ALUMINUM  
ALLOY

Joseph H. Brennan, Niagara Falls, N. Y., assignor  
to Union Carbide and Carbon Corporation, a  
corporation of New York

No Drawing. Application April 20, 1949,  
Serial No. 88,681

1 Claim. (Cl. 75—134)

1

The invention relates to a low-carbon ferrochromium-silicon-aluminum alloy.

The alloy of the invention is particularly useful in the production of low-carbon ferrochromium or chromium steels by the reduction of chromium ore or chromium-bearing slags. Its use results in a more complete recovery of chromium than has heretofore been possible by the use of ferrochrome-silicon and ferrosilicon alloys. A further advantage of the new alloy is that less lime is required as a flux to neutralize silica resulting from the reduction of chromium ores or oxide. This latter advantage results from the conversion of the aluminum content of the alloy to alumina which is a neutral substance, or weak base, in reactions involving the reduction of chromium oxide.

According to the invention the new alloy contains between 10% and 45% chromium, between 35% and 55% silicon, between 5% and 25% aluminum, carbon in an amount less than 0.1%, the remainder being substantially all iron.

In order to demonstrate the advantages of the alloy of the invention comparative tests were made under identical conditions, wherein low-carbon ferrochromium was prepared from chromite by reduction with a commercial ferrochromium-silicon alloy and the alloy of the invention, respectively. It was observed that in the tests employing a ferrochromium-silicon alloy containing 50% silicon, remainder iron and chromium, a slag containing 5 to 7% chromium resulted; whereas in the tests employing the alloy of the invention containing in addition to iron and chromium, approximately 40% silicon and

2

10% aluminum the resulting slag contained only 2 to 3% chromium.

The alloy of the invention may be made in any of several ways as for example by a simple melting together of the constituent metals, or by carbon reduction with a mixture of ferrochromium, quartzite and clay or bauxite, or by direct complete carbon reduction of chromite and quartzite. This last method is described and 10 claimed in a co-pending application, Serial No. 88,684, filed April 20, 1949, in the name of August M. Kuhlmann. When the alloy is prepared by this method a minor proportion of calcium may be present depending upon the concentration of lime in the raw materials. The addition of calcium to the alloy is often beneficial in the usual 15 applications for which the alloy is used.

What is claimed is:

20 A ferrochromium-silicon-aluminum alloy containing chromium between 10% and 45%, silicon between 35% and 55%, aluminum between 5% and 25%, the remainder iron and incidental impurities, carbon being present in an amount less than 0.1%.

25

JOSEPH H. BRENNAN.

## REFERENCES CITED

30 The following references are of record in the file of this patent:

## UNITED STATES PATENTS

| Number       | Name    | Date          |
|--------------|---------|---------------|
| 2,031,947    | Haglund | Feb. 25, 1936 |
| 35 2,203,214 | Doom    | June 4, 1940  |